



US005616455A

**United States Patent**

[19]

**Murphy**[11] **Patent Number:** **5,616,455**[45] **Date of Patent:** **Apr. 1, 1997**

[54] **METHOD OF PREPARATION OF A MONODISPersed TABULAR SILVER HALIDE GRAIN EMULSION**

[75] Inventor: **Martin D. Murphy**, Savona, Italy

[73] Assignee: **Imation Corp.**, Woodbury, Minn.

[21] Appl. No.: **605,574**

[22] Filed: **Feb. 22, 1996**

[30] **Foreign Application Priority Data**

Mar. 29, 1995 [EP] European Pat. Off. .... 95104630

[51] **Int. Cl.<sup>6</sup>** ..... **G03C 1/015**

[52] **U.S. Cl.** ..... **430/569**

[58] **Field of Search** ..... 430/569

[56] **References Cited**

U.S. PATENT DOCUMENTS

|           |         |               |       |         |
|-----------|---------|---------------|-------|---------|
| 4,184,877 | 1/1980  | Maternaghan   | ..... | 430/567 |
| 4,301,241 | 11/1981 | Saito         | ..... | 430/569 |
| 4,386,156 | 5/1983  | Mignot        | ..... | 430/567 |
| 4,425,426 | 1/1984  | Abbott et al. | ..... | 430/502 |
| 4,722,886 | 2/1988  | Nottorf       | ..... | 430/569 |
| 4,797,354 | 1/1989  | Saitou et al. | ..... | 430/567 |
| 4,798,775 | 1/1989  | Yagi et al.   | ..... | 430/569 |
| 4,801,522 | 1/1989  | Ellis         | ..... | 430/569 |
| 4,945,037 | 7/1990  | Saitou        | ..... | 430/567 |
| 4,952,489 | 8/1990  | Arnicucci     | ..... | 430/569 |
| 4,977,074 | 12/1990 | Saitou        | ..... | 430/567 |
| 5,013,641 | 5/1991  | Buntaine      | ..... | 430/569 |
| 5,028,521 | 7/1991  | Grzeskowiak   | ..... | 430/569 |
| 5,087,555 | 2/1992  | Saitou        | ..... | 430/569 |
| 5,215,879 | 6/1993  | Suzuki et al. | ..... | 430/569 |
| 5,254,453 | 10/1993 | Chang         | ..... | 430/569 |
| 5,318,888 | 6/1994  | Weberg et al. | ..... | 430/569 |

FOREIGN PATENT DOCUMENTS

0503700A1 9/1992 European Pat. Off. .... G03C 1/07

|           |         |                    |       |            |
|-----------|---------|--------------------|-------|------------|
| 0513722A1 | 11/1992 | European Pat. Off. | ..... | G03C 1/07  |
| 0513723A1 | 11/1992 | European Pat. Off. | ..... | G03C 1/07  |
| 0513724A1 | 11/1992 | European Pat. Off. | ..... | G03C 1/07  |
| 0513725A1 | 11/1992 | European Pat. Off. | ..... | G03C 1/07  |
| 0569075A1 | 11/1993 | European Pat. Off. | ..... | G03C 1/005 |
| 0577886A1 | 1/1994  | European Pat. Off. | ..... | G03C 1/005 |
| 0588338A1 | 3/1994  | European Pat. Off. | ..... | G03C 1/005 |

*Primary Examiner*—Mark F. Huff  
*Attorney, Agent, or Firm*—Mark A. Litman; Gregory A. Evaratt

[57] **ABSTRACT**

The present invention relates to a method for the preparation of a tabular silver halide grain emulsion, wherein said silver halide emulsion comprises tabular grains having a thickness lower than 0.5  $\mu\text{m}$  and an average aspect ratio of at least 2:1 accounting for at least 50% of the total projected area, and shows a coefficient of variation lower than 30%, said method comprising the steps of (a) forming silver halide nuclei by adding from 5% to 15% by weight of total silver nitrate to a reaction vessel comprising a dispersing medium and bromide aqueous solution at a pBr ranging from 0 to 2 and a pH ranging from 2 to 5, (b) performing a first addition of a silver halide solvent after at least 50% by weight of silver nitrate used during nucleation has been added, (c) ripening the silver halide nuclei, (d) growing said silver halide nuclei by double jet addition of a soluble silver salt and a soluble bromide salt aqueous solutions at pBr between 1 and 2 to obtain tabular silver halide grains, (e) adjusting the pBr to a value ranging from 4.5 and 7 by single jet addition of a soluble silver salt aqueous solution, (f) performing a second addition of silver halide solvent, and (g) thickening said tabular silver halide grains by double jet addition of a soluble silver salt and a soluble bromide salt aqueous solutions at pBr between 1.0 and 3.0.

**9 Claims, No Drawings**

**METHOD OF PREPARATION OF A  
MONODISPERSED TABULAR SILVER  
HALIDE GRAIN EMULSION**

**FIELD OF THE INVENTION**

The present invention relates to a process for preparing monodispersed tabular silver halide emulsion useful in light-sensitive photographic materials.

**BACKGROUND OF THE INVENTION**

Tabular silver halide grains, their preparation and use in photographic emulsions, are widely known. Tabular silver halide grains are crystals possessing two major faces that are substantially parallel. They have been extensively studied in the literature since photographic emulsions containing these grains appeared to offer some significant advantages over photographic emulsions containing round or globular or cubic grains. Tabular grains usually have polygonal (i.e., triangular or hexagonal) parallel crystal faces, each of which is usually greater than any other crystal face of the grain and are conventionally defined by their aspect ratio (namely AR) which is the ratio of the diameter of the grain to the thickness. Tabular grains offer significant technical and commercial advantages apparent to those skilled in the art. The most important advantages of tabular grains can be summarized as follows:

1. Tabular grains have a high surface to volume ratio so that a large amount of sensitizing dye can be adsorbed on the surface, and a high development rate and covering power can be obtained.
2. Tabular grains tend to lie parallel to the surface of the support base when emulsions containing them are coated and dried so that it is possible to reduce the thickness of the coated layer and accordingly to increase sharpness.
3. When a sensitizing dye is added to tabular grains, the extinction coefficient of the dye is greater than the extinction coefficient for the indirect transition of the silver halide so that in X-ray materials it is possible to obtain a relevant reduction in cross-over, thereby preventing any worsening of quality.
4. Tabular grains are usually very thin and so the amount of radiation absorbed per grain (proportional to the thickness) is low and there is low fogging due to natural radiation on aging.
5. Tabular grains show low light scattering and the images obtained from them have a high resolution.

In spite of all these advantages, tabular grain emulsions tend toward more dispersed grain populations than can be achieved in the preparation of conventional silver halide grains. This has been a concern since reducing grain dispersion or variation in grain size within an emulsion is a basic approach to increasing the imaging consistency of the emulsion. Grain dispersion concern relates to (1) the presence of non-conforming grain shapes, such as, for example, octahedral, cubic, or rod shapes and (2) to the variance of the grain size distribution. Non-conforming grains can interact differently with light and exhibit some undesirable properties. For example, faces of non-tabular grains are randomly oriented with respect to the support base, octahedral grains exhibit lower covering power and greater thickness, and rod grains can self develop in the absence of light, thereby increasing fog.

On the other hand, even a population of grains having a common shape can have a high dispersion in terms of grain size distribution. A common method for quantifying grain size distribution is to extract a sample of individual grains, calculate the corresponding diameter for each grain ( $D_{1 \rightarrow n}$ , wherein n is the number of extracted grains), calculate the average diameter ( $D_m = \sum_{1 \rightarrow n} D/n$ ), calculate the standard deviation of the grain population diameters (S), divide the standard deviation (S) by the average diameter (Dm) and multiply by 100, thereby obtaining the coefficient of variation (COV) of the grain population as a percentage.

It is known in the art that emulsions having a low COV (e.g., lower than 30%) can be optimally sensitized as a result of their similar surface areas, have low light scattering and therefore a high image sharpness as a result of the reduction of the finer grain population, have a low granularity as a result of the reduction of the larger grain population, and have a higher contrast.

Accordingly, various solutions have been proposed in the art to reduce the COV of tabular grain emulsions. Monodispersed tabular grain emulsions and methods to prepare them are disclosed for example in U.S. Pat. No. 4,150,994, U.S. Pat. No. 4,184,877, U.S. Pat. No. 4,184,878, U.S. Pat. No. 4,301,241, U.S. Pat. No. 4,386,156, U.S. Pat. No. 4,400,463, U.S. Pat. No. 4,425,426, U.S. Pat. No. 4,797,354, U.S. Pat. No. 4,977,074, U.S. Pat. No. 4,945,037, U.S. Pat. No. 5,215,879, U.S. Pat. No. 4,798,775, U.S. Pat. No. 4,722,886, U.S. Pat. No. 4,801,522, U.S. Pat. No. 5,013,641, U.S. Pat. No. 5,254,453, EP 503,700, EP 569,075, EP 577,886, EP 588,338, EP 600,753. These patents and patent applications attempt to obtain monodispersed tabular grains by controlling various parameters during nucleation and ripening of the silver halide emulsion. The most important nucleation conditions to be kept under control for obtaining monodispersed tabular grain emulsions are temperature, gelatin concentration, addition rates of silver salt solution, addition rates of alkali halide solution, stirring rate, iodide content in the alkali halide solution, amount of silver halide solvent, pH of the dispersing medium, concentration of bromide ions in the reaction vessel, molecular weight of dispersing medium, iodide content in the vessel at the start, and the like. Similarly, the most important ripening conditions are temperature, dispersing medium concentration, silver halide solvent concentration, pBr, and addition rates of silver salt solution.

Maternaghan in U.S. Pat. No. 4,150,994, U.S. Pat. No. 4,184,877, and U.S. Pat. No. 4,184,878 describes the formation of thick monodispersed tabular grain emulsion from seed crystals having at least 90%mol of iodide.

Saito in U.S. Pat. No. 4,301,241 describes a process for forming a silver halide emulsion containing multiple twin crystal grains and a narrow grain size distribution. The examples report multiple twin crystal grain silver bromoiodide emulsions having an average grain size from 0.86 to 1.023  $\mu\text{m}$  and a coefficient of variation of from 11.6% to 13.6%.

Mignot in U.S. Pat. No. 4,386,156 describes silver bromide tabular grain emulsions having an aspect ratio of at least 8.5:1 and a COV of less than 30. The tabular grains described by Mignot are bounded by (100) crystal faces and are square or rectangular.

Abbot et al. in U.S. Pat. No. 4,425,426 disclose a radiographic element comprising tabular grain emulsion in which grains having thickness lower than 0.2  $\mu\text{m}$ , and average aspect ratio from 5:1 to 8:1, account for at least 50% of the total projected area. During precipitation of silver halide grains the rate of introduction of silver and halide salts is

maintained below the threshold level at which the formation of new grain nuclei is favored in order to obtain relatively monodispersed thin tabular grains with COV lower than 30%.

Saitou et al. in U.S. Pat. No. 4,797,354 disclose a silver halide emulsion comprising hexagonal tabular grains with an "adjacent edge ratio" of from 2/1 to 1/1 accounting for 70% to 100% of the projected area of all the grains, and further that said hexagonal tabular grains are monodisperse and have an average aspect ratio from 2.5:1 to 20:1. The term "adjacent edge ratio" is referred to as the ratio of the longest edge length to the shortest edge length of each hexagonal tabular grain. Accordingly, the definition of "adjacent edge ratio" is a measure of the hexagon regularity.

Saitou et al. U.S. Pat. No. 4,977,074 disclose and claim a silver halide emulsion comprising substantially circular tabular grains with a "linear ratio" equal to or lower than 2/5 accounting for from 70% to 100% of the projected area of all the grains, and further that said circular tabular grains are monodispersed. The term "linear ratio" is defined as the ratio of the total length of the linear portion in the substantially circular tabular grain divided by the total length of the extrapolated hexagonal tabular grain. The lower the linear ratio value, the more circular the grain.

U.S. Pat. No. 4,945,037 discloses a process to produce a tabular silver halide grain emulsion in which at least 60% of the total projected area is covered by tabular grains having a core portion and an outer portion, the iodide content of the core portion being from 7 mol % to the solid solution limit. The process is characterized by specific nucleating condition, that is, a gelatin concentration of from 0.1 to 20% by weight, an addition rate of silver and halide salts of from  $6 \times 10^{-4}$  to  $2.9 \times 10^{-1}$  mol/minute per liter, and a pBr value of from 1.0 to 2.5.

U.S. Pat. No. 4,798,775 discloses a process to obtain monodispersed tabular grains comprising the steps of forming silver halide nuclei with a silver iodide content of from 0 to 5% in the mother liquor, by maintaining the pBr in the reaction vessel between 2.0 and -0.7 for at least the initial half of the nucleation time, ripening the nuclei formed in the nucleation step by maintaining the concentration of silver halide solvent from  $10^{-4}$  to 5 moles per liter of mother liquor, and growing the seed grains by addition of silver and halide soluble salts or by addition of fine silver halide grains.

U.S. Pat. No. 4,801,522 discloses a process to form tabular silver halide grains having a thickness of from 0.05 to 0.5  $\mu\text{m}$ , average grain volume of from 0.05 to 1.0  $\text{mm}^3$  and a mean aspect ratio higher than 2:1 comprising the steps of adding silver nitrate to a reaction vessel comprising a bromide ion concentration of from 0.08 to 0.25N (pBr=1.1-0.6), adding ammonia solution to achieve 0.002 to 0.2N after at least 2% of the total silver has been added to the vessel, and adding silver and halide (Br or BrI) salts by balanced double jet.

U.S. Pat. No. 4,722,886 describes a process to form a monodispersed tabular silver halide grain emulsion comprising the steps of adding silver nitrate to a reaction vessel comprising a bromide ion concentration of from 0.08 to 0.25N to form silver halide nuclei, adding a basic silver halide solvent (e.g., ammonia solution) to achieve 0.02 to 0.2N after at least 2% by weight of the total silver has been added to the vessel, stopping silver nitrate addition for a time period of from 0.5 to 60 minutes at a Br ion concentration of from 0.005 to 0.05N, neutralizing at least part of the present solvent, and growing the formed silver halide grains by adding silver and halide (Br or BrI) soluble salts by balanced double jet.

U.S. Pat. No. 5,013,641 describes a process of forming monodispersed silver halide emulsions comprising (a) combining silver nitrate and sodium bromide in gelatin solution, (b) adding NaOH to adjust the pH to greater than 9, (c) allowing digestion of the nucleated particles, (d) adjusting the pH to below 7 by acid addition, and (e) adding silver nitrate and sodium halide to grow the nucleated particles.

U.S. Pat. No. 5,254,453 discloses a process for forming monodispersed silver bromide or bromoiodide grains with COV lower than 25%, thickness of from 0.05 to 0.5  $\mu\text{m}$ , mean aspect ratio higher than 2, and diameter of from 0.2 to 3  $\mu\text{m}$  comprising the following steps: (a) digesting the nucleated particles in a basic silver halide solvent at a concentration of from 0.0015 to 0.015N and (b) neutralizing said basic solvent after digestion and before growing.

EP 503,700 discloses a process of forming monodispersed silver bromide or bromoiodide tabular emulsions with a COV lower than or equal to 15% characterized by the addition of an aminoazaindene at any stage of the preparation, but before 50% of the total silver halide is precipitated.

EP 569,075 discloses a process of forming monodispersed silver bromide or bromoiodide tabular emulsions with average aspect ratio higher than 2, an average thickness of from 0.15 and 0.30  $\mu\text{m}$ , and a COV of from 0.15 to 0.45 wherein the process is characterized by (a) providing a gelatin/bromide solution at a pBr of from 1.0 to 2.0, (b) nucleating by consuming less than 10% of the total silver nitrate used, (c) a first double jet growth (consuming at least 10% of the total silver nitrate used) at a pBr value of from 1.0 and 2.5, and (d) a second double jet growth (consuming at least 40% of the total silver nitrate used) at a pBr value higher than 2.7

EP 577,886 describes a process of forming monodispersed silver bromide or bromoiodide tabular emulsions with average-aspect ratio of from 2 to 8, and a COV lower than 30. The process comprises the following steps: (a) performing a nucleation step by balanced double jet by precipitating at most 5% of the total silver halide, (b) ripening the formed nuclei, (c) performing at least one growing step by balanced double jet at pBr lower than 2, (d) ultrafiltrating the reaction mixture during the precipitation steps with an ultrafiltration flux equal to or greater than the sum of the flow rates of the silver and halide ion solutions.

Grzeskowiak, in U.S. Pat. No. 5,028,521, discloses a process for preparing monodispersed tabular silver halide grain emulsions having an aspect ratio from 3:1 to 12:1 consisting in (a) preparing a bromide/gelatin mixture at pBr of from 0.7 to 1.0, (b) adding silver nitrate and further halide to maintain excess of bromide, (c) adding ammonia to achieve at least 0.05N after at least 20% by weight of the total silver is added, (d) adding further silver nitrate and halide by balanced double jet, by maintaining an ammonia concentration of at least 0.03N.

EP 588,338 describes a process characterized by specific nucleating condition, that comprises (a) adding from 0.30 to 9.0% by weight of the total amount of soluble silver salt to a vessel containing 0.08 to 0.25M aqueous soluble halide salt (b) adding a solution of ammoniacal base when 0.30 to 9% by weight of the total amount of soluble silver salt has been added, (c) adding soluble silver salt to obtain growth pBr of from 1.3 to 2.3, and (d) adding soluble silver and halide salts to grow tabular grains

Other recent patents and patent applications attempt to obtain monodispersed silver halide tabular emulsion by adding a specific polymeric surfactant during nucleation and/or ripening.

U.S. Pat. No. 5,215,879 describes a process to obtain monodispersed silver halide emulsions in which a polymer

having the following formula is added during the ripening step.



wherein Y is H or carboxyl group; R<sub>1</sub> is H, a halogen atom, an alkyl group or CH<sub>2</sub>COOM, where M is H or an alkali metal atom; L is —CONH—, —NHCO—, —COO—, OCO—, —CO—, or —O—; J is an alkylene group, an arylene group, or (CH<sub>2</sub>CH<sub>2</sub>O)<sub>m</sub>(CH<sub>2</sub>)<sub>n</sub>, where m is an integer from 0 to 40 and n is an integer from 0 to 4; and Q is H, alkyl group, a N-containing heterocyclic group, a quaternary ammonium group, a dialkylamino group, OM, —NH<sub>2</sub>, —SO<sub>3</sub>M, —O—PO<sub>3</sub>M<sub>2</sub> and —CO—R.

EP 513,722, EP 513,723, EP 513,724, and EP 513,725 describe a process in which monodispersed tabular emulsions are obtained by adding, during nucleation, polymers having the following general formulas (1) to (4), respectively.

- (1) LAO-HAO-LAO
- (2) HAO-LAO-HAO
- (3) HAO-LAO-L-LAO-HAO
- (4) LAO-HAO-L-HAO-LAO

wherein LAO is a lipophilic alkylene oxide block unit, HAO is a hydrophilic alkylene oxide block unit, and L is a trivalent or tetravalent organic group comprising nitrogen.

#### SUMMARY OF THE INVENTION

The present invention relates to a new method for the preparation of a tabular silver halide grain emulsion, wherein said silver halide emulsion comprises tabular grains having a thickness lower than 0.5 μm and an average aspect ratio of at least 2:1 accounting for at least 50% of the total projected area, and shows a coefficient of variation lower than 30%, said method comprising the following steps:

- (a) forming silver halide nuclei by adding from 5% to 15% by weight of total silver nitrate to a reaction vessel comprising a dispersing medium and bromide aqueous solution at a pBr ranging from 0 to 2 and a pH ranging from 2 to 5,
- (b) performing a first addition of a silver halide solvent after at least 50% by weight of silver nitrate used during nucleation has been added,
- (c) ripening the silver halide nuclei,
- (d) growing said silver halide nuclei by double jet addition of a soluble silver salt and a soluble bromide salt aqueous solutions at pBr between 1 and 2 to obtain tabular silver halide grains,
- (e) adjusting the pBr to a value ranging from 4.5 and 7 by single jet addition of a soluble silver salt aqueous solution,
- (f) performing a second addition of silver halide solvent, and
- (g) thickening said tabular silver halide grains by double jet addition of a soluble silver salt and a soluble bromide salt aqueous solutions at pBr between 1.0 and 3.0.

#### DETAILED DESCRIPTION OF THE INVENTION

The present invention relates to a method for the preparation of a tabular silver halide grain emulsion, wherein said

silver halide emulsion comprises tabular grains having a thickness lower than 0.5 μm and an average aspect ratio of at least 2:1 accounting for at least 50% of the total projected area, and shows a coefficient of variation lower than 30%, said method comprising the following steps:

- (a) forming silver halide nuclei by adding from 5% to 15% by weight of total silver nitrate to a reaction vessel comprising a dispersing medium and bromide aqueous solution at a pBr ranging from 0 to 2 and a pH ranging from 2 to 5,
- (b) performing a first addition of a silver halide solvent after at least 50% by weight of silver nitrate used during nucleation has been added,
- (c) ripening the silver halide nuclei,
- (d) growing said silver halide nuclei by double jet addition of a soluble silver salt and a soluble bromide salt aqueous solutions at pBr between 1 and 2 to obtain tabular silver halide grains,
- (e) adjusting the pBr to a value ranging from 4.5 and 7 by single jet addition of a soluble silver salt aqueous solution,
- (f) performing a second addition of silver halide solvent, and
- (g) thickening said tabular silver halide grains by double jet addition of a soluble silver salt and a soluble bromide salt aqueous solutions at pBr between 1.0 and 3.0.

#### GRAIN PREPARATION

Tabular silver halide grains contained in the silver halide emulsions of the present invention have an average diameter:thickness ratio (often referred to in the art as aspect ratio) of at least 2:1, preferably 2:1 to 20:1, more preferably 2:1 to 14:1, and most preferably 2:1 to 8:1. Average diameters of the tabular silver halide grains suitable for use in this invention range from about 0.3 to about 5 μm, preferably 0.5 to 3 μm, more preferably 0.8 to 1.5 μm. The tabular silver halide grains suitable for use in this invention have a thickness of less than 0.5 μm, more preferably within 0.1 to 0.45 μm.

The tabular silver halide grain dimensions and characteristics described above can be readily ascertained by procedures well-known to those skilled in the art. The term "diameter" is defined as the diameter of a circle having an area equal to the projected area of the grain. The term "thickness" means the distance between two substantially parallel main planes constituting the tabular silver halide grains. From the measure of diameter and thickness of each grain the diameter:thickness ratio of each grain can be calculated, and the diameter:thickness ratios of all tabular grains can be averaged to obtain their average diameter:thickness ratio. By this definition the average diameter:thickness ratio is the average of individual tabular grain diameter:thickness ratios. In practice, it is simpler to obtain an average diameter and an average thickness of the tabular grains and to calculate the average diameter:thickness ratio as the ratio of these two averages. Whatever the method used, the average diameter:thickness ratios obtained do not greatly differ.

The projected area of the tabular silver halide grains obtained with the process of the present invention accounts for at least 50%, preferably at least 80% and more preferably at least 90% of the projected area of all the silver halide grains of the emulsion. The coefficient of variation of the

tabular grain emulsion obtained with the process of the present invention is lower than 30%, preferably lower than 25%, and more preferably lower than 20%.

In the present invention, commonly employed halogen compositions of the silver halide grains can be used. Typical silver halides include silver chloride, silver bromide, silver iodide, silver chloroiodide, silver bromoiodide, silver chlorobromoiodide and the like. However, silver bromide and silver bromoiodide are preferred silver halide compositions for tabular silver halide grains with silver bromoiodide compositions containing from 0 to 10 mol % silver iodide, preferably from 0.2 to 5 mol % silver iodide, and more preferably from 0.5 to 1.5% mol silver iodide. The halogen composition of individual grains may be homogeneous or heterogeneous.

The preparation process of a silver halide emulsion generally comprises a nucleation step, in which silver halide grain seeds are formed, followed by one or more growing steps, in which the grain seeds achieve their final dimension, and a washing step, in which all soluble salts are removed from the final emulsion. A ripening step is usually present between the nucleation and growing step and/or between the growing and the washing steps.

According to the process of the present invention, an aqueous solution of a dispersing medium is put in a reaction vessel together with a bromide salt aqueous solution. The dispersing medium initially present in the reaction vessel can be chosen among those conventionally employed in the silver halide emulsions. Preferred dispersion media include hydrophilic colloids, such as proteins, protein derivatives, cellulose derivatives (e.g. cellulose esters), gelatin (e.g. acid or alkali treated gelatin), gelatin derivatives (e.g. acetylated gelatin, phthalated gelatin and the like), polysaccharides (e.g. dextran), gum arabic, casein and the like. It is also common to employ said hydrophilic colloids in combination with synthetic polymeric binders and peptizers such as acrylamide and methacrylamide polymers; polymers of alkyl and sulfoalkyl acrylates and methacrylates, polyvinyl alcohol and its derivatives, polyvinyl lactams, polyamides, polyamines, polyvinyl acetates, and the like. The bromide salt is typically a water soluble salt of alkaline or alkaline earth metals, such as, for example, sodium bromide, potassium bromide, ammonium bromide, calcium bromide, or magnesium bromide.

The temperature of the reaction vessel content is preferably in the range of from 30° C. to 80° C., more preferably from 40° C. to 70° C. The pH of the starting solution ranges from 2 to 5, preferably from 3 to 5. The pBr of the starting solution ranges from 0 to 2, preferably from 0.2 to 1.0.

During the nucleation step (a), a silver nitrate aqueous solution is added by single jet method to the reaction vessel at a constant flow rate ranging from 5 to 30 ml/min, preferably from 10 to 20 ml/min, by maintaining the temperature constant. During the nucleation step, the amount of silver nitrate added is from 5 to 15% by weight of total silver nitrate. According to the present invention, the term "total silver nitrate" means the amount of silver nitrate employed during the overall emulsion making process, that is, from step (a) to (g). After at least 50%, preferably after at least 70%, and more preferably after at least 90% by weight of silver nitrate used during nucleation has been added, a silver halide solvent is added to the reaction vessel. The silver halide solvent is chosen amongst any conventionally known silver halide solvents, e.g., thiourea, ammonia, thioether, thiosulfate or thiocyanate. The concentration of the silver halide solvent into the reaction vessel after the addition can

range from 0.002 to 0.3N, preferably from 0.02 to 0.2N. According to a preferred embodiment, the silver halide solvent is an ammonia aqueous solution.

At the end of the nucleation step, the addition of silver nitrate is stopped and the obtained silver halide seed grains are subjected to the ripening step (c). The silver halide seeds are allowed to ripen at a temperature of from 30° to 80° C., preferably from 50° to 80° C., for a period of time ranging from 1 to 20 minutes, preferably from 1 to 15 minutes, in the presence of the silver halide solvent. At the end of the ripening step, the pH of the reaction vessel content is adjusted to a value of from 4.5 to 5.5, preferably of about 5.

After that, the silver halide seed grains are subjected to a growth step (d) by double jet addition of a silver nitrate aqueous solution and a halide salt aqueous solution at accelerated flow rate, with a linear ramp starting from within 5 to 15 ml/min and rising to within 50 to 100 ml/min, preferably starting from within 5 to 10 ml/min and rising to within 70 to 90 ml/min. The halide salt aqueous solution added during this step can either comprise bromide ions or a mixture of bromide and iodide and/or chloride ions. The pBr of the reaction vessel content is kept under control at a value of from 1 to 2, preferably from 1.2 to 1.8. During this growth step (d), the amount of silver nitrate added is from 45 to 55% based on the total weight silver nitrate employed.

At the end of the growing step (d), the pBr is adjusted to a value of from 4.5 to 7, preferably from 5 to 6.5 by single jet addition of a silver nitrate solution. During this step (e), the amount of silver nitrate used is from 5 to 15% based on the total weight silver nitrate employed. At the end of the silver nitrate addition, a second addition (f) of silver halide solvent is performed to give a concentration of from 0.002 to 0.3N, preferably from 0.02 to 0.2N.

The thickening step (g) is performed by a second double jet addition of silver nitrate and halide salt aqueous solutions at a constant flow rate of from 5 to 30 ml/min, preferably from within 10 to 20 ml/min. The halide salt aqueous solution added during this step can either comprise bromide ions or a mixture of bromide and iodide and/or chloride ions. During this second growth step, the amount of silver nitrate added is from 20 to 30% based on the total weight silver nitrate employed. During the thickening step, the pBr value is kept under control at a value of from 1 to 3, preferably from 1.5 to 2.5.

If during the growing and thickening steps, a soluble iodide salt is added together with the bromide salt the amount of the iodide present in the final emulsion ranges from 0.01 to 10%mol, preferably from 0.05 to 5%mol based on the total halide content. If a soluble chloride salt is added, the amount of the chloride present in the final emulsion ranges from 1 to 20%mol, preferably from 5 to 10%mol based on the total halide content.

At the end of the thickening step (g), the tabular grains can optionally be further ripened for a period of time of from 1 to 20 minutes.

At the end of silver halide grain precipitation, water soluble salts are removed from the emulsion by procedures known in the art. Suitable cleaning arrangements are those wherein the dispersing medium and soluble salts dissolved therein can be removed from the silver halide emulsion on a continuous basis, such as, for example, a combination of dialysis or electrodialysis for the removal of soluble salts or a combination of osmosis or reverse osmosis for the removal of the dispersing medium.

In a particularly preferred embodiment, among the known techniques for removing the dispersing medium and soluble

salts while retaining silver halide grains in the remaining dispersion, ultrafiltration is a particularly advantageous cleaning arrangement for the practice of this process. Typically, an ultrafiltration unit comprising membranes of inert, non-ionic polymers is used as a cleaning arrangement. Since silver halide grains are large in comparison with the dispersing medium and the soluble salts or ions, silver halide grains are retained by said membranes while the dispersing medium and the soluble salts dissolved therein are removed.

The action mechanism of preferred membranes is described in GB 1,307,331. The membranes used in the ultrafiltration comprise a very thin layer of extremely fine pore texture supported upon a thicker porous structure. Suitable membranes consist of polymers such as polyvinylacetate, polyvinylalcohol, polyvinylformate, polyvinylethers, polyamides, polyimides, polyvinyl chloride and polyvinylidene chloride, aromatic polymers, such as aromatic polyesters, polytetrafluoroethylene, regenerated cellulose, cellulose esters, such as cellulose acetate, or mixed cellulose esters. The membranes in question have anisotropic, semipermeable properties, show considerable mechanical, thermal and chemical stability and are photographically inert. The membranes are preferably permeable to molecules having molecular weights of up to about 300,000 and, more especially, of up to about 50,000.

#### CHEMICAL SENSITIZATION

Prior to use, the tabular silver halide grain emulsion prepared according to the method of the present invention is generally fully dispersed and bulked up with gelatin or other dispersion of peptizer and subjected to any of the known methods for achieving optimum sensitivity.

Chemical sensitization is performed by adding chemical sensitizers and other additional compounds to the silver halide emulsion, followed by the so-called chemical ripening at high temperature for a predetermined period of time. Chemical sensitization can be performed by various chemical sensitizers such as gold, sulfur, reducing agents, platinum, selenium, sulfur plus gold, and the like. The tabular silver halide grains for use in the present invention, after grain formation and desalting, are chemically sensitized by at least one gold sensitizer and at least one thiosulfonate sensitizer. During chemical sensitization other compounds can be added to improve the photographic performances of the resulting silver halide emulsion, such as, for example, antifoggants, stabilizers, optical sensitizers, supersensitizers, and the like.

Gold sensitization is performed by adding a gold sensitizer to the emulsion and stirring the emulsion at high temperature of preferably 40° C. or more for a predetermined period of time. As a gold sensitizer, any gold compound which has an oxidation number of +1 or +3 and is normally used as gold sensitizer can be used. Preferred examples of gold sensitizers are chloroauric acid, the salts thereof and gold complexes, such as those described in U.S. Pat. No. 2,399,083. It is also useful to increase the gold sensitization by using a thiocyanate together with the gold sensitizer, as described, for example, in T. H. James, *The Theory of the Photographic Process*, 4th edition, page 155, published by MacMillan Co., 1977. Specific examples of gold sensitizers include chloroauric acid, potassium chloroaurate, auric trichloride, sodium aurithiosulfate, potassium

aurithiocyanate, potassium iodoaurate, tetracyanoauric acid, 2-aurosulfobenzothiazole methochloride and ammonium aurothiocyanate.

Thiosulfonate sensitization is performed by adding a thiosulfonate sensitizer to the tabular silver halide emulsion and stirring the emulsion at a high temperature of 40° C. or more for a predetermined period of time.

The amounts of the gold sensitizer and the thiosulfonate sensitizer for use in the present invention change in accordance with the various conditions, such as activity of the gold and thiosulfonate sensitizer, type and size of tabular silver halide grains, temperature, pH and time of chemical ripening. These amounts, however, are preferably from 1 to 20 mg of gold sensitizer per mol of silver, and from 1 to 100 mg of thiosulfonate sensitizer per mol of silver. The temperature of chemical ripening is preferably 45° C. or more, and more preferably 50° C. to 80° C. The pAg and pH may take arbitrary values.

During chemical sensitization, addition times and order of gold sensitizer and thiosulfonate sensitizer are not particularly limited. For example, gold and thiosulfonate sensitizers can be added at the initial stage of chemical sensitization or at a later stage either simultaneously or at different times. Usually, gold and thiosulfonate sensitizers are added to the tabular silver halide emulsion by their solutions in water, in a water-miscible organic solvent, such as methanol, ethanol and acetone, or as a mixture thereof.

#### SPECTRAL SENSITIZATION

The tabular silver halide emulsions of the present invention are preferably spectrally sensitized. It is specifically contemplated to employ in the present invention, in combination with the tabular silver halide emulsions, spectral sensitizing dyes having absorption maxima in the blue, minus blue (i.e., green and red) and infrared portions of the electromagnetic spectrum. Spectral sensitizing dyes for use in the present invention include polymethine dyes, such as cyanine and complex cyanine dyes, merocyanine and complex merocyanine dyes, as well as other dyes, such as oxonols, hemioxonols, styryls, merostyryls and streptocyanines as described by F. M. Hamer, *The Cyanine and Related Compounds*, Interscience Publishers, 1964.

The cyanine dyes include, joined by a methine linkage, two basic heterocyclic nuclei, such as pyrrolidine, oxazoline, thiazoline, pyrrole, oxazole, thiazole, selenazole, tetrazole and pyridine and nuclei obtained by fusing an alicyclic hydrocarbon ring or an aromatic hydrocarbon ring to each of the above nuclei, such as indolenine, benzindolenine, indole, benzoxazole, naphthoxazole, benzothiazole, naphthothiazole, benzoselenazole, benzimidazole and quinoline. These nuclei can have substituents groups.

The merocyanine dyes include, joined by a methine linkage, a basic heterocyclic nucleus of the type described above and an acid nucleus, such as a 5- or 6-membered heterocyclic nucleus derived from barbituric acid, 2-thiobarbituric acid, rhodanine, hydantoin, 2-thiohydantoin, 4-thiohydantoin, 2-pyrazolin-5-one, 2-isoxazolin-5-one, indan-1, 3-dione, cyclohexane-1,3-dione, and isoquinolin-4-one.

Of the above dyes, dyes most effectively used in the present invention are cyanine dyes, such as those represented by the following formula:



wherein n, m, p and d each independently represents 0 or 1, L represents a methane linkage, e.g.,  $=\text{CH}-$ ,  $\equiv\text{C}(\text{C}_2\text{H}_5)$ , etc., R1 and R2 each represents a substituted or unsubstituted alkyl group, preferably a lower alkyl group of from 1 to 4 carbon atoms, e.g., methyl, ethyl, propyl, butyl, cyclohexyl and dodecyl, a hydroxyalkyl group, e.g., b-hydroxyethyl and W-hydroxybutyl, an alkoxyalkyl group, e.g., b-methoxyethyl and W-butoxyethyl a carboxyalkyl group, e.g., b-carboxyethyl and W-carboxybutyl sulfatoalkyl group, e.g., b-sulfatoethyl and W-sulfatobutyl, an acyloxyalkyl group, e.g., b-acetoxyethyl, g-acetoxypropyl and W-butyroloxybutyl, an alkoxy-carbonylalkyl group, e.g., b-methoxycarbonylethyl and W-ethoxycarbonylbutyl, benzyl, phenethyl, or an aryl group of up to 30 carbon atoms, e.g., phenyl, tolyl, xylyl, chlorophenyl and naphthyl, X represents an acid anion, e.g., chloride, bromide, iodide, thiocyanate, sulfate, perchlorate, p-toluenesulfonate and methylsulfate; said methine linkage forming an intramolecular salt when p is 0; Z1 and Z2, the same or different, each represents the non metallic atoms necessary to complete the same simple or condensed 5- or 6-membered heterocyclic nucleus, such as a benzothiazole nucleus (e.g., benzothiazole, 3-, 5-, 6- or 7-chlorobenzothiazole, 4-, 5- or 6-methylbenzothiazole, 5- or 6-bromobenzothiazole, 4- or 5-phenyl-benzothiazole, 4-, 5- or 6-methoxybenzothiazole, 5, 6-dimethyl-benzothiazole and 5- or 6-hydroxy-benzothiazole), a naphthothiazole nucleus (e.g., a-naphthothiazole, b-naphthothiazole, 5-methoxy-b-naphthothiazole, 5-ethoxy-a-naphthothiazole and 8-methoxy-a-naphthothiazole), a benzoselenazole nucleus (e.g., benzoselenazole, 5-chloro-benzoselenazole and tetrahydrobenzoselenazole), a naphthoselenazole nucleus (e.g., a-naphtho-selenazole and b-naphthoselenazole), a benzoxazole nucleus (e.g., benzoxazole, 5- or 6-hydroxybenzoxazole, 5-chloro-benzoxazole, 5- or 6-methoxy-benzoxazole, 5-phenylbenzoxazole and 5,6-dimethyl-benzoxazole), a naphthoxazole nucleus (e.g., a-naphthoxazole and b-naphthoxazole), a 2-quinoline nucleus (e.g., 2-quinoline, 6-, 7-, or 8-methyl-2-quinoline, 4-, 6- or 8-chloro-2-quinoline, 5-, 6- or 7-ethoxy-2-quinoline and 6- or 7-hydroxy-2-quinoline), a 4-quinoline nucleus (e.g., 4-quinoline, 7- or 8-methyl-4-quinoline and 6-methoxy-4-quinoline), a benzimidazole nucleus (e.g., benzimidazole, 5-chloro-benzimidazole and 5, 6-dichloro-benzimidazole), a thiazole nucleus (e.g., 4- or 5-methyl-thiazole, 5-phenyl-thiazole and 4,5-di-methyl-thiazole), an oxazole nucleus (e.g., 4- or 5-methyl-oxazole, 4-phenyl-oxazole, 4-ethyl-oxazole and 4,5-dimethyl-oxazole), and a selenazole nucleus (e.g., 4-methyl-selenazole and 4-phenyl-selenazole). More preferred dyes within the above class are those having an internal salt group and/or derived from benzoxazole and benzimidazole nuclei as indicated before. Typical methine spectral sensitizing dyes for use in the present invention include those listed below.



The methine spectral sensitizing dyes for use in this invention are generally known in the art. Particular reference can be made to U.S. Pat. Nos. 2,503,776, 2,912,329, 3,148,187, 3,397,060, 3,573,916 and 3,822,136 and FR Pat. No. 1,118,778. Also their use in photographic emulsions is very known wherein they are used in optimum concentrations corresponding to desired values of sensitivity to fog ratios. Optimum or near optimum concentrations of spectral sen-

sitzing dyes in the emulsions of the present invention generally go from 10 to 500 mg per mol of silver, preferably from 50 to 200, more preferably from 50 to 100.

Spectral sensitizing dyes can be used in combinations which result in supersensitization, i.e., spectral sensitization which is greater in a spectral region than that from any concentration of one dye alone or which would result from an additive effect of the dyes. Supersensitization can be obtained with selected combinations of spectral sensitizing dyes and other addenda, such as stabilizers and antifoggants, development accelerators and inhibitors, optical brighteners, surfactants and antistatic agents, as described by Gilman, *Photographic Science and Engineering*, 18, pp. 418-430, 1974 and in U.S. Pat. Nos. 2,933,390, 3,635,721, 3,743,510, 3,615,613, 3,615,641, 3,617,295 and 3,635,721.

Preferably, spectral sensitizing dyes are used in supersensitizing combination with polymeric compounds containing an aminoallylidene-malononitrile ( $>\text{N}-\text{CH}=\text{CH}-\text{CH}=(\text{CN})_2$ ) moiety, as those described in U.S. Pat. No. 4,307,183. Said polymeric compounds are preferably obtained upon copolymerization of an allyl monomer which has an ethylenically condensed aminoallylidene-malononitrile moiety (such as diallylaminooallylidene-malononitrile monomer therein with an ethylenically unsaturated monomer, said monomer being preferably a water-soluble monomer; said copolymerization being preferably a solution polymerization said polymeric compound being preferably a water-soluble polymer; said monomer more preferably being an acrylic or methacrylic monomer, most preferably being acrylamide or acrylic acid.

Examples of polymeric compounds which can be used in supersensitizing combination with spectral sensitizing dyes are preferably the polymeric compounds described in the following Table B wherein the monomer is copolymerized (in solution in the presence of a polymerization initiator) with a diallylaminooallylidene-malononitrile monomer, as well as a weight percent quantity of aminoallylidene-malononitrile moieties (AAMN) within the polymers themselves are indicated.

TABLE B

| Compound | Monomer                     | % AAMN |
|----------|-----------------------------|--------|
| 1        | Acrylamide                  | 9      |
| 2        | Methacrylic acid            | 11     |
| 3        | Acrylamide                  | 10.5   |
| 4        | Acrylic acid                | 23     |
| 5        | Acrylamide                  | 44     |
| 6        | Vinylpirrolidone            | 44     |
| 7        | Vinyloxazolidone            | 14.5   |
| 8        | Vinyloxazolidone            | 37     |
| 9        | Methacrylamide              | 8      |
| 10       | Acrylamide-Allylamide.HCl   | 10     |
| 11       | Acrylamide-Diallylamide.HCl | 7      |

Methods of preparation of said polymeric compounds are described in the above mentioned U.S. Pat. No. 4,307,183. The optimum concentrations of said polymeric compounds generally go from 10 to 1,000 mg per mol of silver, preferably from 50 to 500, more preferably from 150 to 350, the weight ratio of the polymeric compound to the spectral sensitizing dye normally being of 10/1 to 1/10, preferably 5/1 to 1/5, more preferably 2.5/1 to 1/1 (such a ratio of course depending upon the aminoallylidene-malononitrile moiety content of the polymeric compound: the higher such content, the lower such ratio).

Spectral sensitization can be performed at any stage of silver halide preparation. It can be performed subsequent to the completion of chemical sensitization or concurrently

with chemical sensitization, or can precede chemical sensitization, or even can commence prior to the completion of silver halide precipitation. In the preferred form, spectral sensitizing dyes can be incorporated in the tabular grain silver halide emulsions prior to chemical sensitization.

#### PHOTOGRAPHIC MATERIAL

The tabular silver halide grain emulsions are useful in light-sensitive photographic materials. A light-sensitive silver halide photographic material can be prepared by coating the above described silver halide emulsion on a photographic support. There is no limitation with respect to the support. Examples of materials suitable for the preparation of the support include glass, paper, polyethylene-coated paper, metals, cellulose nitrate, cellulose acetate, polyesters such as polyethylene terephthalate, polyethylene, polypropylene and other well-known supports.

Said light-sensitive silver halide photographic material specifically is applicable to light-sensitive photographic color materials such as color negative films, color reversal films, color papers, etc., as well as black-and-white light-sensitive photographic materials such as X-ray light-sensitive materials, lithographic light-sensitive materials, black-and-white photographic printing papers, black-and-white negative films, etc.

Preferred light-sensitive silver halide photographic materials are X-ray light-sensitive materials comprising the above described silver halide emulsion coated on one surface, preferably on both surfaces of a support, preferably a polyethylene terephthalate support. Preferably, the silver halide emulsion is coated on the support at a total silver coverage comprised in the range of 3 to 6 grams per square meter. Usually, the X-ray light-sensitive materials are associated with intensifying screens so as to be exposed to radiation emitted by said screens. The screens are made of relatively thick phosphor layers which transform the X-rays into light radiation (e.g., visible light). The screens absorb a portion of X-rays much larger than the light-sensitive material and are used to reduce the X-ray dose necessary to obtain a useful image. According to their chemical composition, the phosphors can emit radiation in the blue, green or red region of the visible spectrum and the silver halide emulsions are sensitized to the wavelength region of the light emitted by the screens. Sensitization is performed by using spectral sensitizing dyes adsorbed on the surface of the silver halide grains as known in the art.

The exposed light-sensitive materials of this invention can be processed by any of the conventional processing techniques. The processing can be a black-and-white photographic processing for forming a silver image or a color photographic processing for forming a dye image depending upon the purpose. Such processing techniques are illustrated for example in Research Disclosure, 17643, December 1978. Roller transport processing in an automatic processor is particularly preferred, as illustrated in U.S. Pat. Nos. 3,025,779, 3,515,556, 3,545,971 and 3,647,459 and in U.K. Pat. No. 1,269,268. Hardening development can be undertaken, as illustrated in U.S. Pat. No. 3,232,761.

The silver halide emulsion layer containing the tabular silver halide grain emulsion obtained with the method of this invention can contain other constituents generally used in photographic products, such as binders, hardeners, surfactants, speed-increasing agents, stabilizers, plasticizers, optical sensitizers, dyes, ultraviolet absorbers, etc., and reference to such constituents can be found, for example, in

Research Disclosure, Vol. 176 (December 1978), pp. 22-28. Ordinary silver halide grains may be incorporated in the emulsion layer containing the tabular silver halide grains as well as in other silver halide emulsion layers of the light-sensitive silver halide photographic material of this invention. Such grains can be prepared by processes well-known in the photographic art.

The present invention is now illustrated by reference to the following examples, which are not intended to limit the scope of the invention.

#### EXAMPLE 1

##### Control emulsion A

An aqueous gelatin solution consisting of 5124 g of water, 45 g of deionized gelatin, 92.3 g of potassium bromide, and 1.83 g of sodium thiocyanate was put in a 10 liter reaction vessel. The starting pBr and pH values were 0.8 and 4.75, respectively.

##### Nucleation

72 ml of a 2N silver nitrate aqueous solution were added over a period of 8 minutes at a constant flow rate, while keeping the temperature constant at 56° C.

##### Growth

1172 ml of a 2N silver nitrate aqueous solution and 1172 ml of a 2N potassium bromide aqueous solution were added to the vessel by accelerated double jet method, with a linear addition ramp rising from 9.00 ml/min to 77.85 ml/min. At the end of the growing step, the pAg value was raised to about 7.8 by a single jet addition of 120 ml of a 2N silver nitrate aqueous solution at a constant rate of 60 ml/min, followed by a single jet addition of a 2N silver nitrate aqueous solution at a constant rate of 14.25 ml/min over a maximum period of 30 minutes.

##### Thickening:

75 ml of a 12N aqueous solution of ammonia were added in the vessel over a period of a minute. After that, 495 ml of a 2N silver nitrate aqueous solution and the corresponding amount of a 1.94N potassium bromide and 0.06N potassium iodide aqueous solution were added over a period of about 30 minutes. The pBr of the reaction vessel was kept constant at a value of about 2.0.

At the end of the tabular silver halide grain formation, water soluble salts were removed from the emulsion by procedures known in the art.

##### Invention emulsion B

An aqueous gelatin solution consisting of 2700 g of water, 60 g of deionized gelatin, and 56.4 g of potassium bromide, was put in a 10 liter reaction vessel. The starting pBr and pH values were 0.77 and 3, respectively.

##### Nucleation

204 ml of a 2N silver nitrate aqueous solution were added over a period of 13 minutes at a constant flow rate of about 15.7 ml/min, while keeping the temperature constant at 56° C. After 10 minutes, 100 ml of a 4.56N ammonia aqueous solution were added to the reaction vessel. At the end of the silver nitrate addition, the silver halide nuclei are ripened for 4 minutes at 56° C., and then the pH was adjusted to 5.

##### Growth

A 2N silver nitrate aqueous solution and the corresponding amount of a 2N potassium bromide aqueous solution were added to the vessel by accelerated double jet method, with a linear addition ramp rising from 9.00 ml/min to 77.85 ml/min over 25.5 minutes, by keeping the pBr value constant at 1.5. At the end of the growing step, the pBr value was adjusted to about 5.6 by a single jet addition of a 2N silver nitrate aqueous solution at a constant rate of 14.25 ml/min over a maximum period of 15 minutes. After that, 75 ml of a 12N aqueous solution of ammonia were added in the vessel over a period of a minute.

stant at 1.5. At the end of the growing step, the pBr value was adjusted to about 5.6 by a single jet addition of a 2N silver nitrate aqueous solution at a constant rate of 14.25 ml/min over a maximum period of 15 minutes. After that, 75 ml of a 12N aqueous solution of ammonia were added in the vessel over a period of a minute.

##### Thickening

A 2N silver nitrate aqueous solution and the corresponding amount of a 1.94N potassium bromide and 0.06N potassium iodide aqueous solution were added over a period of about 30 minutes at a constant flow rate of a 6.5 ml/min. The pBr of the reaction vessel was kept constant at a value of about 2.0.

At the end of the tabular silver halide grain formation, water soluble salts were removed from the emulsion by procedures known in the art.

##### Invention emulsion C

An aqueous gelatin solution consisting of 2700 g of water, 60 g of deionized gelatin, and 56.4 g of potassium bromide, was put in a 10 liter reaction vessel. The starting pBr and pH values were 0.77 and 4.75, respectively.

##### Nucleation

204 ml of a 2N silver nitrate aqueous solution were added over a period of 13 minutes at a constant flow rate of about 15.7 ml/min, while keeping the temperature constant at 56° C. After 10 minutes, 100 ml of a 4.56N ammonia aqueous solution were added to the reaction vessel. At the end of the silver nitrate addition, the silver halide nuclei are ripened for 4 minutes at 56° C., and then the pH was adjusted to 5.

##### Growth

A 2N silver nitrate aqueous solution and the corresponding amount of a 2N potassium bromide aqueous solution were added to the vessel by accelerated double jet method, with a linear addition ramp rising from 9.00 ml/min to 77.85 ml/min over 25.5 minutes, by keeping the pBr value constant at 1.5. At the end of the growing step, the pBr value was adjusted to about 5.6 by a single jet addition of a 2N silver nitrate aqueous solution at a constant rate of 14.25 ml/min over a maximum period of 15 minutes. After that, 75 ml of a 12N aqueous solution of ammonia were added in the vessel over a period of a minute.

##### Thickening

A 2N silver nitrate aqueous solution and the corresponding amount of a 1.94N potassium bromide and 0.06N potassium iodide aqueous solution were added over a period of about 30 minutes at a constant flow rate of a 6.5 ml/min. The pBr of the reaction vessel was kept constant at a value of about 2.0.

At the end of the tabular silver halide grain formation, water soluble salts were removed from the emulsion by procedures known in the art.

##### Invention emulsion D

An aqueous gelatin solution consisting of 2700 g of water, 60 g of deionized gelatin, and 56.4 g of potassium bromide, was put in a 10 liter reaction vessel. The starting pBr and pH values were 0.77 and 3.00, respectively.

##### Nucleation

204 ml of a 2N silver nitrate aqueous solution were added over a period of 13 minutes at a constant flow rate of about 15.7 ml/min, while keeping the temperature constant at 56° C. After 13 minutes, 100 ml of a 4.56N ammonia aqueous solution were added to the reaction vessel. At the end of the silver nitrate addition, the silver halide nuclei are ripened for 4 minutes at 56° C., and then the pH was adjusted to 5.

## Growth

A 2N silver nitrate aqueous solution and the corresponding amount of a 2N potassium bromide aqueous solution were added to the vessel by accelerated double jet method, with a linear addition ramp rising from 9.00 ml/min to 77.85 ml/min over 25.5 minutes, by keeping the pBr value constant at 1.5. At the end of the growing step, the pBr value was adjusted to about 4.8 by a single jet addition of a 2N silver nitrate aqueous solution at a constant rate of 14.25 ml/min over a maximum period of 15 minutes. After that, 75 ml of a 12N aqueous solution of ammonia were added in the vessel over a period of a minute.

## Thickening

A 2N silver nitrate aqueous solution and the corresponding amount of a 1.94N potassium bromide and 0.06N potassium iodide aqueous solution were added over a period of about 30 minutes at a constant flow rate of about 6.5 ml/min. The pBr of the reaction vessel was kept constant at a value of about 2.0.

At the end of the tabular silver halide grain formation, water soluble salts were removed from the emulsion by 20 procedures known in the art.

The resulting tabular grain emulsions A to D showed the characteristics exposed in the following Table 1.

TABLE 1

|                      | Control<br>Emul-<br>sion A | Invention<br>Emul-<br>sion B | Invention<br>Emul-<br>sion C | Invention<br>Emul-<br>sion D |
|----------------------|----------------------------|------------------------------|------------------------------|------------------------------|
| Average Diameter     | 1.20 $\mu\text{m}$         | 1.10 $\mu\text{m}$           | 1.15 $\mu\text{m}$           | 1.23 $\mu\text{m}$           |
| Average Thickness    | 0.20 $\mu\text{m}$         | 0.28 $\mu\text{m}$           | 0.44 $\mu\text{m}$           | 0.44 $\mu\text{m}$           |
| Average Aspect Ratio | 6.00                       | 3.92                         | 2.61                         | 2.79                         |
| Standard Deviation   | 0.48 $\mu\text{m}$         | 0.32 $\mu\text{m}$           | 0.27 $\mu\text{m}$           | 0.24 $\mu\text{m}$           |
| COV                  | 40%                        | 29%                          | 23.5%                        | 19.5                         |

The data of Table 1 clearly shows the improvement of the process of the present invention in obtaining a tabular silver halide emulsion having a reduced aspect ratio and a lower coefficient of variation.

I claim:

1. Method for the preparation of a tabular silver halide grain emulsion, wherein said silver halide emulsion comprises tabular grains having a thickness lower than 0.5  $\mu\text{m}$  and an average aspect ratio of at least 2:1 accounting for at least 50% of the total projected area, and shows a coefficient of variation lower than 30%, said method comprising the following steps:

5  
10  
15

(a) forming silver halide nuclei by adding from 5% to 15% by weight of total silver nitrate to a reaction vessel comprising a dispersing medium and bromide aqueous solution at a pBr ranging from 0 to 2 and a pH ranging from 2 to 5

(b) performing a first addition of a silver halide solvent after at least 50% by weight of silver nitrate used during nucleation has been added

(c) ripening the silver halide nuclei

(d) growing said silver halide nuclei by double jet addition of a soluble silver salt and a soluble bromide salt aqueous solutions at pBr between 1 and 2 to obtain tabular silver halide grains

(e) adjusting the pBr to a value ranging from 4.5 to 7 by single jet addition of a soluble silver salt aqueous solution

(f) performing a second addition of silver halide solvent

(g) thickening said tabular silver halide grains by double jet addition of a soluble silver salt and a soluble bromide salt aqueous solutions at pBr between 1.0 and 3.0.

25. The method according to claim 1, wherein said silver halide emulsion shows a coefficient of variation lower than 25%.

30. The method according to claim 1, wherein the pBr value of said nucleation step (a) ranges from 0.2 to 1.0.

35. The method according to claim 1, wherein said silver halide solvent is added after at least 90% by weight of silver nitrate used during said nucleation step (a) has been added.

40. The method according to claim 1, wherein the concentration of silver halide solvent in the reaction vessel ranges from 0.002 to 0.3N.

45. The method according to claim 1, wherein said silver halide solvent is ammonia.

50. The method according to claim 1, wherein the pBr value of said growing step (d) ranges from 1.2 to 1.8.

55. The method according to claim 1, wherein the pBr value of said step (e) is adjusted to a value ranging from 5.0 to 6.5.

60. The method according to claim 1, wherein the pBr value of said thickening step (g) ranges from 1.5 to 2.5.

\* \* \* \* \*